

# UNITED STATES PATENT OFFICE.

WILLIAM H. KEMLER AND CHARLES H. GREENE, OF PITTSBURG, PENNSYLVANIA.

## METHOD OF MANUFACTURING MINERAL WOOL.

SPECIFICATION forming part of Letters Patent No. 637,126, dated November 14, 1899.

Application filed June 30, 1897. Serial No. 642,942. (No specimens.)

*To all whom it may concern:*

Be it known that we, WILLIAM H. KEMLER and CHARLES H. GREENE, of Pittsburg, county of Allegheny, and State of Pennsylvania, have 5 invented a new and useful Improvement in the Manufacture of Mineral Wool, of which the following is a full, clear, and exact description.

Our invention relates to the making of mineral wool by subjecting slag to a blast of steam, air, or other fluid; and its object is to provide a simple and inexpensive process whereby such a wool may be obtained which is substantially free from sulfur.

15 Heretofore in the manufacture of mineral wool the rock mixture or blast-furnace slag has been melted in a cupola-furnace and has contained sulfur or sulfurous compounds in considerable amounts, this sulfur being derived from the sulfur in the coke used in such furnaces. When said wool is employed for covering metal surfaces, it has been found that the sulfur or sulfurous compounds therein combined with the metal and corroded and 25 injured it.

Our invention does away with this injurious element or compound in the wool; and it consists in passing flame or gases which are substantially free from sulfur over a silicious 30 rock mixture which is free from sulfur, thereby producing a molten bath of slag which is free from sulfur, and then blowing this slag into wool in the ordinary manner.

In carrying out our improved process in its 35 preferred form we take a silicious material, such as ordinary Ligonier block, and melt it in a reverberatory or other suitable tank or hearth furnace, using sufficient limestone or other suitable flux to form a liquid bath. 40 This Ligonier block is a well-known silicious stone containing about twenty per cent. of lime. The mixture may be heated from any

suitable source of heat in which the solid fuel is kept out of contact with the mixture, and we prefer to use natural gas, which is substantially free from sulfur, though we have found that producer-gas, which contains sulfur in small quantities, may be used without giving any substantial amount of sulfur in the wool. An oil-burner or other heating means may be 45 employed within the scope of our invention, provided the flame or gases are substantially free from sulfur or contain it in such minute quantities as to not materially affect the quality of the product. After the mass has been 50 melted in this manner it is tapped out and blown into wool in the ordinary manner, the wool thus produced being substantially free from sulfur or deleterious sulfur compounds.

Instead of using a silicious material with 55 alkaline earth or other suitable fluxes a self-fluxing rock or sand may be used, and we intend to cover the same in our claim, and many other variations may be made in the materials employed for the bath and the fur- 60 nace used without departing from our invention, since

We claim—

The method of manufacturing mineral wool, consisting in passing a flame or gas, substantially free from sulfur, over a mixture of silicious material and a flux, substantially free from sulfur, thereby producing a molten bath of slag with substantially no sulfur, and then blowing this slag into wool, substantially 65 as described.

In testimony whereof we have hereunto set our hands.

WILLIAM H. KEMLER.  
CHARLES H. GREENE.

Witnesses:

F. E. GAITHER,  
C. BYRNES.